

## UNITED STATES PATENT OFFICE

2,104,269

## METAL PLATING

Floyd F. Oplinger, Niagara Falls, N. Y., assignor  
to E. I. du Pont de Nemours & Company, Wil-  
mington, Del., a corporation of Delaware

No Drawing. Application April 17, 1934.  
Serial No. 721,000

6 Claims. (Cl. 204—13)

This invention relates to the art of electroplating and more particularly to the production of decorative electroplated articles.

An object of the present invention is to produce certain decorative effects on metal by electroplating, as hereinafter described. Other objects will appear in the following description.

In my copending application Ser. No. 709,171 filed Jan. 31, 1934 I have described and claimed a method of producing smooth, bright coatings of electroplated coatings which comprises electroplating a metal with a metal coating having a lower melting point than that of the base metal and thereafter subjecting the plated article to a heat treatment under non-oxidizing conditions, at a temperature above the melting point of the plated metal.

I have discovered that when an electroplated coating which has been heat treated at a temperature above its melting point is subsequently repated, preferably with a coating of the same metal or an alloy thereof, the final electroplated coating is deposited in the form of spangle-like crystals which have a decorative effect pleasing to the eye. These spangled coatings are of a crystalline nature and resemble the ordinary galvanized iron made by coating metal sheet in a bath of molten zinc.

I have further discovered that the spangled effect can be produced by plating over coatings of such metals as tin, lead or zinc or their alloys which coatings have been applied to the base metal in the molten state.

According to one method of practicing my invention, I first electroplate a metallic article to be decorated with a metal having a melting point lower than that of the base metal of which the article is constructed. For example I may plate an iron, steel, copper or brass article with such metals as tin, cadmium, zinc or suitable alloys of these metals. For the purposes of this invention, the electroplated coating may be made of any desired thickness. After the metal has been plated, it is washed and dried and then heated for a short time under non-oxidizing conditions at a temperature above the melting point of the electroplated metal, so as to fuse the latter without fusing the base metal. One convenient method of carrying out this step is to dip the electroplated article in a bath of molten tallow or other suitable liquid maintained at the required temperature. For example, a tin coating may be treated by dipping the plated article into a bath of molten tallow maintained at a temperature of 450—500° C. for 10 seconds to 2

minutes, depending on the size of the article. Various other means of heating under non-oxidizing conditions will be apparent. For example, the article may be heated in an atmosphere of a non-oxidizing gas such as hydrogen or 5 nitrogen.

After heating, the article is suitably cooled preferably at a controlled rate, since the rate of cooling affects the ultimate result as hereinafter explained. Various known methods of controlled 10 cooling may be used, e. g. by dipping in oil or water.

After cooling, the heat treated article is again plated with the metal with which it was first plated. This second electrodeposit is produced 15 in a bright crystalline form, having the spangled effect above described. If desired, the spangled coating may be converted to a smooth or mirror-like coating by heat treating as above described under non-oxidizing conditions above the melting 20 point of the plate. If this is done, the resulting heat treated article may again be plated with the result that the spangled coating is again reproduced.

In some cases, especially when applying my 25 invention to the decoration of cold-rolled steel sheet and similar steel articles, it is preferable to utilize a method for preliminary treatment of the article to be decorated which is described and claimed in my copending application S. N. 30 709,171. In accordance with the method, I first clean the metal surface by known means to remove oil, grease and the like. The cleaned metal article then is treated with a strong acid solution until a visible and uniformly etched surface is 35 produced. This etching process should be continued until the etching of the metal is plainly visible to the unaided eye, so that the treated surface presents a more or less uniformly dull appearance. Various strong acids, for example 40 sulfuric acid, hydrochloric acid, nitric acid or various mixtures of such strong acids may be used for this etching process. It is preferable to have the acid solution warm, for example to 120—160° F. 45

After the article has been suitably etched, it is rinsed with water and then it is treated in an alkaline solution for a few minutes. Various solutions of strong alkali are suitable for this treatment; it is often preferable to have substantial quantities of alkali metal cyanide present in the alkaline bath used for treating the metal. Preferably I treat the metals in the alkaline bath by using the alkaline solution as an electrolyte and making the article to be treated the 50 55

anode. After the alkaline treatment, the article is plated, heat-treated and repleted as described above, to produce the decorative effect.

If the above mentioned etching process has been too drastic, the surface of the plated metal may have a somewhat dull appearance after the heat treatment; when a less drastic etching is used, the article will have a smooth, mirror-like surface. However, for the purposes of the present invention it is immaterial whether the degree of etching is the minimum required to produce a smooth surface on heat treating or whether it is so drastic as to produce a dull surface by the heating step. In either case a satisfactory decorative result is obtained.

The following examples illustrate more specifically methods of carrying out my invention:

*Example 1*

20 Sheet copper was treated with a warm mixture of sulfuric and nitric acid solutions until visibly and uniformly etched. The etched copper was plated with tin from an alkaline electrolyte. The plated sheet then was immersed in a bath of 25 molten tallow maintained at a temperature of 240-260° C. until the tin plate was fused and then cooled by quenching with water. The sheet was then cooled and repleted with tin. The second electrodeposit of tin had a beautiful, crystalline or spangled appearance, similar to that of galvanized iron sheet.

*Example 2*

35 Cold rolled steel sheet was cleaned to remove grease and dirt, pickled in strong sulfuric acid until visibly etched, washed with water and given an anodic treatment for about 3 minutes in an alkaline solution of sodium cyanide at a temperature of 140-160° F. The steel sheet then was 40 plated with tin, heat treated and repleted as described in Example 1, with substantially the same results.

*Example 3*

45 A coating of spangled tin was produced on cold rolled sheet steel by the method of Example 2. The spangled sheet then was electroplated with gold to a good color. The resulting gold plate accurately reproduced the underlying crystal pattern.

*Example 4*

50 Cold-rolled steel was treated by the method described in Example 2, except that the initial plate was a tin alloy, electroplated from an alkaline tin bath to which was added a salt of the alloy constituent, i. e., cadmium or zinc. After heating the alloy-plated sheet under non-oxidizing conditions above the melting point of the plate and cooling, the sheet was repleted with 55 pure tin from an alkaline electrolyte. The alloys used for the initial plate were tin-cadmium and tin-zinc. Various decorative effects were obtained, with different crystal patterns, depending on the rate of cooling after heat treatment 60 of the initial plate.

65 In utilizing my process for producing the spangled effect on cold-rolled steel, it is preferable that the base metal be visibly etched with acid and then treated with an alkali as hereinbefore described, prior to the initial plating. In any case, I prefer to visibly etch the base metal with acid and then treat with alkali prior to applying the first coating.

70 Various modifications of my invention will be 75 apparent. For example, the final electroplated

coating may be identical with the underlying coating, an alloy of the same or a different metal. For example, a base metal having a fused coating of tin may be repleted to produce the spangled effect by replingating the tin with tin alloy or 5 with another metal such as copper or gold. I prefer to replete with the same metal as is used for the under coat or an alloy thereof. In some cases where the final coating is a different metal than the underlying coating it is advantageous to 10 produce the spangled effect by the herein described method before the final coating is applied. For example, I may coat a metal with a fused tin coating either by hot dipping in molten tin or by first electroplating and then heating 15 the electroplated tin to a temperature above its melting point and then replingating this fused tin coating with tin or tin alloys to produce a spangled tin final coat. This final coat then may be plated with another metal such as copper or gold, 20 with the result that the final coat will show substantially the same crystalline structure as the spangled tin on which it was plated. Various metals may be used as the initial coating; I prefer to use tin or a tin alloy.

25 The appearance of the final coat will depend upon a number of factors. For example, by using different metals or alloys for the first coat, different decorative effects may be obtained. Also, the rate at which the first coat is cooled 30 after having been fused often will affect the size of the crystals appearing in the final coat; in general, if the rate of cooling is rapid the crystals appearing in the final electrodeposit will be small, while slow cooling promotes the formation of 35 large crystals. Also, preliminary treatment of the base metal prior to application of the initial coating, e. g. by etching with acid, also will influence the crystalline appearance of the final electrodeposit. In general, the crystalline patterns may be made more definite by a visible 40 etching of the base metal prior to the application of the first coating.

45 The appearance of the final products also will depend to some extent upon the thickness of the final coating. If the coating is too thick, the desired spangled effect may not appear; that is, if sufficient metal is electrodeposited, the crystalline appearance which is at first formed may finally become obliterated. Hence, to obtain the 50 best results the final coating should be relatively thin. The degree of thinness required, however, will vary with different metals. For example, when copper or gold is plated over a fused or spangled tin coating, the final coating must be 55 very thin, while on the other hand, a final electrodeposit of tin or tin alloy may be as much as 0.0003 inch or more in thickness without obliterating the crystalline appearance.

I claim:

1. A process for decorating metal surfaces comprising providing a metal surface with a coating of fused tin and thereafter electroplating said fused coating with a sufficiently thin layer of tin to develop a spangled coating.

2. A process for decorating metal surfaces comprising providing a metal surface with an oxide-free coating of fused tin and thereafter electroplating said fused coating with a sufficiently thin layer of tin to develop a spangled coating 70 and finally electrodepositing on said spangled coating a thin layer of gold.

3. A process for decorating a metal surface comprising electroplating said surface with tin, heating the electroplated surface under non- 75

oxidizing conditions to a temperature above the melting point of the electrodeposit, cooling and thereafter electroplating said surface with a sufficiently thin layer of tin to develop a spangled coating.

4. A process for decorating a metal surface comprising treating said surface with an acid until the surface thereof is at least visibly etched, coating said etched surface with a fused layer of tin and thereafter electroplating said surface with a sufficiently thin layer of tin to develop the spangled coating.

5. A process for decorating a cold-rolled steel surface comprising treating said surface with an acid until the surface thereof is at least visibly etched, following with an alkaline treatment, electroplating said etched surface with tin, heating the electroplated surface under non-oxidizing conditions to a temperature above the melting point of the electrodeposit, cooling, thereafter electroplating said surface with tin to produce a spangled coating and finally electrodepositing on said spangled coating a thin layer of gold.

6. A process for decorating a cold-rolled steel surface comprising treating said surface with an acid until the surface thereof is at least visibly etched, following with an alkaline treatment, electroplating said etched surface with tin, heating the electroplated surface under non-oxidizing conditions to a temperature above the melting point of the electrodeposit, cooling and thereafter electroplating said surface with a sufficiently thin layer of metal to develop a spangled coating.

5

6. A process for decorating a cold-rolled steel surface comprising treating said surface with an acid until the surface thereof is at least visibly etched, following with an alkaline treatment, electroplating said etched surface with tin, heating the electroplated surface under non-oxidizing conditions to a temperature above the melting point of the electrodeposit, cooling, thereafter electroplating said surface with tin to produce a spangled coating and finally electrodepositing on said spangled coating a thin layer of gold.

FLOYD F. OPLINGER.

CERTIFICATE OF CORRECTION.

Patent No. 2,104,269.

January 4, 1938.

FLOYD F. OPLINGER.

It is hereby certified that error appears in the printed specification of the above numbered patent requiring correction as follows: Page 3, second column, line 4, claim 5, for the word "metal" read tin; and that said Letters Patent should be read with this correction therein that the same may conform to the record of the case in the Patent Office.

Signed and sealed this 22nd day of February, A. D. 1938.

(Seal)

Henry Van Arsdale,  
Acting Commissioner Of Patents.

oxidizing conditions to a temperature above the melting point of the electrodeposit, cooling and thereafter electroplating said surface with a sufficiently thin layer of tin to develop a spangled coating.

4. A process for decorating a metal surface comprising treating said surface with an acid until the surface thereof is at least visibly etched, coating said etched surface with a fused layer of tin and thereafter electroplating said surface with a sufficiently thin layer of tin to develop the spangled coating.

5. A process for decorating a cold-rolled steel surface comprising treating said surface with an acid until the surface thereof is at least visibly etched, following with an alkaline treatment, electroplating said etched surface with tin, heating the electroplated surface under non-oxidizing conditions to a temperature above the melting point of the electrodeposit, cooling, thereafter electroplating said surface with tin to produce a spangled coating and finally electrodepositing on said spangled coating a thin layer of gold.

6. A process for decorating a cold-rolled steel surface comprising treating said surface with an acid until the surface thereof is at least visibly etched, following with an alkaline treatment, electroplating said etched surface with tin, heating the electroplated surface under non-oxidizing conditions to a temperature above the melting point of the electrodeposit, cooling and thereafter electroplating said surface with a sufficiently thin layer of metal to develop a spangled coating.

5

6. A process for decorating a cold-rolled steel surface comprising treating said surface with an acid until the surface thereof is at least visibly etched, following with an alkaline treatment, electroplating said etched surface with tin, heating the electroplated surface under non-oxidizing conditions to a temperature above the melting point of the electrodeposit, cooling, thereafter electroplating said surface with tin to produce a spangled coating and finally electrodepositing on said spangled coating a thin layer of gold.

FLOYD F. OPLINGER.

CERTIFICATE OF CORRECTION.

Patent No. 2,104,269.

January 4, 1938.

FLOYD F. OPLINGER.

It is hereby certified that error appears in the printed specification of the above numbered patent requiring correction as follows: Page 3, second column, line 4, claim 5, for the word "metal" read tin; and that said Letters Patent should be read with this correction therein that the same may conform to the record of the case in the Patent Office.

Signed and sealed this 22nd day of February, A. D. 1938.

(Seal)

Henry Van Arsdale,  
Acting Commissioner Of Patents.

CERTIFICATE OF CORRECTION.

Patent No. 2,104,269.

January 4, 1938.

FLOYD F. OPLINGER.

It is hereby certified that error appears in the printed specification of the above numbered patent requiring correction as follows: Page 3, second column, line 4, claim 5, for the word "metal" read tin; and that said Letters Patent should be read with this correction therein that the same may conform to the record of the case in the Patent Office.

Signed and sealed this 22nd day of February, A. D. 1938.

Henry Van Arsdale,  
Acting Commissioner Of Patents.

(Seal)